

1

3,165,375

**PROCESS OF CHEMICALLY MODIFYING PROTEINACEOUS MATERIALS WITH AZIRIDINE COMPOUNDS AND PRODUCTS THEREOF**

Giuliana C. Tesoro, Dobbs Ferry, N.Y., assignor to J. P. Stevens & Co., Inc., New York, N.Y., a corporation of Delaware

No Drawing. Filed Apr. 25, 1961, Ser. No. 105,285  
20 Claims. (Cl. 8—127.6)

The present invention relates to a method of chemically modifying proteinaceous materials and to the products thereby obtained, and more particularly polypeptide fibers so as to modify the physicochemical properties of said materials and increase their usefulness. Although the invention has particular application to the treatment of wool in the form of fibers, threads, yarns, fabrics and wool waste, it is also applicable to polypeptides generally, including, in addition to wool, other keratins (such as camel hair, mohair, horse hair, hog bristles, human hair, feathers, and horn), silk fibers, collagen, gelatin, leather, synthetic polypeptides and the like.

The application of the present invention for the shrinkproofing and feltproofing of keratin fibers, and especially wool, is of particular interest, since it is well known that the tendency of woolen textiles to shrink and felt in the course of normal laundering procedures severely restricts the use of wool in the textile industry.

Much research has been undertaken with the object of improving the dimensional stability and felting properties of animal fibers, and several methods are known by which the shrinkage of woolen textiles can be reduced. Previously known methods have serious shortcomings, and have therefore been used to a limited extent only. For example, the dimensional stability of wool can be enhanced by treatment with oxidizing agents, but the tensile strength of the wool fiber is severely impaired by such treatments. It is also known to subject wool fibers to alkylation by treating first with a reducing agent which converts the disulfide linkages (—S—S—) to thiol linkages (—SH) and thereafter treating with a polyfunctional halide whereby the thiol groups are linked through new chemical bonds (—S-alkylene-S—). The conditions required for carrying out this reaction are not easily controlled, and although treated wool of good dimensional stability can be obtained by these known processes, the fibers are weakened by the initial reduction reaction and by the alkaline reagents which must be used as acid acceptors in the alkylation reaction. Generally, processes requiring the conversion of disulfide linkages to thiol as shown above, have similar shortcomings, since the reduction reaction disrupts the fiber structure and impairs fiber properties. Furthermore, the processes which are based on reactions of the disulfide linkage can be applied only to sulfur-containing polypeptides, such as wool, but not to those proteins in which disulfide bonds are absent.

In an effort to overcome the disadvantages of the processes indicated above, other treatments have also been developed. For example, the treatment of protein fibers with various types of resins has been suggested, but the deposition of resin on or within protein fibers invariably results in an undesirable stiffening of the fibers, and harshness of hand in the textiles and fabrics manufactured from them. The amount of resin required to achieve the

2

desired results is large, and the insolubilization of the resin which is achieved by a polymerization reaction on or in the fiber requires curing at elevated temperature, leading to discoloration and other undesirable side effects.

5 On the other hand, polyfunctional reactants which can combine chemically with the unmodified protein (such as, for example, the dicarboxylic acid azides described in U.S. Patent 2,881,046) without significant polymerization and which are effective in decreasing the solubility of the protein by crosslinking the polypeptide chains, produce only an insignificant decrease in fabric shrinkage even when the amount of reagent combined is large.

Accordingly it would be highly desirable to provide a chemical process whereby the physicochemical properties of proteinaceous materials and particularly in the form of fibers, threads, yarns and fabrics are enhanced and improved.

15 It is, therefore, an object of this invention to provide a novel process for improving the overall dimensional stability of proteinaceous materials particularly in the form of fibers, threads, yarns and fabrics.

20 A further object of this invention is to provide a novel process for shrinkproofing and feltproofing keratin fibers and particularly wool.

25 A further object of this invention is to provide a novel process whereby improved physicochemical properties are imparted to proteinaceous materials, particularly in the form of fibers, threads, yarns and fabrics, under mild reaction conditions and without requiring a pretreatment of said materials.

30 A further object of this invention is to provide a novel process of imparting shrinkproofing and feltproofing of keratin fibers, and particularly wool, without producing undesirable side effects such as discoloration, harshness, and a reduction in strength of said fibers.

35 A further object of this invention is to provide novel products derived from the aforementioned novel process.

These and other objects of this invention will be apparent from the description which follows.

40 According to the present invention it has been discovered that the solubility properties and the dimensional stability of polypeptides generally, and of keratin fibers in particular can be modified in a highly desirable manner by treatment with certain polyfunctional compounds, which combine chemically with the polypeptide molecule under exceedingly mild conditions without requiring prior reduction or other pretreatment, without adversely affecting the strength of the fiber, and without causing any discoloration, harshening or other undesirable side effects.

45 50 More specifically the novel process of this invention comprises reacting a polypeptide, and preferably a protein fiber, with a polyfunctional aziridine compound which can be represented by a generic Formula I

(I)



55 60 in which  $R_1$ ,  $R_2$ , and  $R_3$  are selected from the group consisting of hydrogen and lower alkyl,  $Q$  can be an organic or inorganic radical the valence of which is equal to  $n$ , and  $n$  has a value of 2 to 3. It has been found that the compounds corresponding to Formula I above have vary-

ing degrees of effectiveness in bringing about the desired results. Compounds in which the nitrogen atoms of the aziridine rings are amino nitrogens are particularly effective. Such polyfunctional amino-aziridines can be represented by a generic Formula II

(II)



in which  $R_1$ ,  $R_2$ ,  $R_3$ , and  $R_4$  are selected from the group consisting of hydrogen and lower alkyl,  $A$  is an organic radical the valence of which is equal to  $n$ , and  $n$  has a value of 2 to 3.

Among the compounds of Formula II, those in which the organic radical  $A$  does not contain reactive groupings are outstanding in their effectiveness. These compounds can be represented by a generic Formula III

(III)



in which the  $R_1$ ,  $R_2$ ,  $R_3$ ,  $R_4$  and  $n$  have the meaning defined above and  $Y$  represents an organic radical the valence of which is equal to  $n$  and which does not contain any reactive functional groups. The preparation and properties of the new compounds represented by generic Formula III are described in copending application No. 94,720, filed on March 10, 1961.

Thus, while it has been found that polyaziridine compounds are generally effective reagents for improving the properties of polypeptide fibers, and particularly wool whether in fiber, thread, yarn or fabric form, those corresponding to the above generic Formula III exhibit greater efficiency than any known compounds, and they can eliminate shrinkage and felting of woolen textiles even when used in very small amounts. Furthermore, the structure of the grouping  $Y$  can be selected so as to maintain a high degree of molecular flexibility in the poly-aziridines and in their reaction products with polypeptides.

Although the reason for the vast superiority of the compounds represented by generic Formulas II and III and particularly of those represented by generic Formula III is not fully understood, it is believed that these compounds possess certain properties which make them singularly suitable for the chemical modification of polypeptide fibers, and that they are unique insofar as they can yield treated products of highly desirable properties under practical conditions, with great efficiency, and in the virtual absence of undesirable side effects.

It also appears that the following important requirements should be fulfilled by reagents employed to enhance the dimensional stability of polypeptide fibers generally, and of wool in particular.

(a) The reagents should possess a functionality greater than one, since by crosslinking of the polymeric molecules within the fiber decreased solubility, increased dimensional stability and increased resilience can be achieved.

(b) The reagents should be capable of forming oligomers and polymers containing reactive end groups, since it is known that monomeric crosslinks are not efficient in preventing the shrinkage and felting of protein fibers. In effect, then, the reagents should be capable of forming polymeric crosslinks within the fiber structure, such crosslinks being attached to the fiber by covalent bonds.

(c) The reagents should possess a high degree of molecular flexibility and internal plasticization, so as to avoid the formation of hard, brittle polymeric compounds in or

on the fiber, since harshness of hand invariably results from the presence of such brittle resins.

(d) The reagents should be capable of reacting under mild conditions of temperature and catalysis, since strongly acidic catalysts, strongly basic catalysts and elevated temperatures are known to cause degradation of protein fibers, and especially of wool.

(e) The reagents should preferably be water soluble, since the use of solvents other than water is hazardous and costly, and aqueous solutions are preferred for industrial processing.

The compounds employed in the process of our invention actually fulfill the above requirements. Examples of compounds which can be used for the process of my invention are:

(a) Amino aziridines prepared from polyfunctional aldehydes by reaction with ethylene imines as shown by way of example in Equation 1

(1)



wherein  $R_1$ ,  $R_2$ ,  $R_3$  are selected from the group consisting of hydrogen and lower alkyl, and  $R$  represents an alkylene radical;

(b) Amino aziridines prepared from polyfunctional epoxy compounds by reaction with ethylene imines as shown by way of example in Equation 2

(2)



wherein  $R_1$ ,  $R_2$ ,  $R_3$  have the meaning defined above, and  $R$  represents a bivalent organic radical;

(c) Amino aziridines prepared by reaction of compounds containing conjugated unsaturation with ethylene imines as shown by way of example in Equation 3

(3)



wherein  $R_1$ ,  $R_2$ ,  $R_3$  have the meaning defined above,  $R_4$  is selected from the group consisting of hydrogen and methyl,  $b$  has a value of zero to 1, and  $R^c$  is an organic radical containing conjugated unsaturation;

(d) Amino aziridines prepared by reaction of compounds containing activated double bonds with ethylene imines as shown by way of example in Equation 4 for

the reaction of divinyl sulfone with ethylene imine (Bessian, Ann. 566, 210-244 (1950))



and in Equation 5 for the reaction of ethylene glycol biscrotonate with ethylene imine



(e) Amino aziridines prepared by reaction of polyfunctional halides with ethylene imines, as described in copending application No. 94,720 filed Mar. 10, 1961, as shown by way of example and in Equation 6



wherein  $\text{R}_1$ ,  $\text{R}_2$ ,  $\text{R}_3$  have the meaning defined above,  $\text{X}$  is halogen and  $\text{R}$  is selected from the group consisting of aralkylene and alkylene radicals. Those compounds in which the radical  $\text{R}$  is a polyalkoxy chain, and which can be represented by a generic Formula IV



in which  $\text{R}_1$ ,  $\text{R}_2$ ,  $\text{R}_3$  have the meaning defined above,  $m$  has a value of 2 to 4, and  $x$  has a value of 1 to 50, are the preferred compounds for the process of my invention since they can be prepared from inexpensive and available raw materials. Moreover, they are water soluble, stable in storage, and react readily with protein fibers under mild conditions. In addition they are extraordinarily effective in eliminating the shrinkage and felting of wool textiles, and their chemical structure is such that their oligomers and polymers (the formation of which is believed to precede the chemical reaction of the aziridine groups with the functional groups of the protein fiber) are not rigid and brittle resins but flexible compounds which allow the full retention of the desirable soft hand of the textiles treated.

In the process of our invention, the protein fibers are treated with a solution, preferably an aqueous solution of the polyfunctional aziridine compound and dried. Drying can be carried out at room temperature or at elevated temperature. After drying, the textile (which can be employed in the form of fiber, yarn, fabric or other textile structure) is allowed to stand at room temperature, or exposed to moderate temperature for a brief period of time until the reaction between polyaziridine and fiber is completed. A mild process wash designed to remove small amounts of residual reagent completes the treatment. Concentrations of reagent varying from about 1% to about 10% can be employed in the treating solution

with concentrations ranging from 2 to 4% giving excellent results. The time required for completing the reaction between aziridine compound and the fiber after the drying step, ranges from a few minutes to several hours, depending on the reactivity of the specific polyaziridine compound and on the reaction temperature. Temperatures ranging from ambient temperatures to about 350° F. can be used but temperatures ranging from ambient temperature to about 300° F. are preferred. Some of the polyaziridine compounds react more rapidly than others. In the case of less reactive compounds, it is sometimes advantageous to carry out the reaction in the presence of a catalytic amount of acid. The addition of acidic material to the treating solution is not usually feasible, since the presence of acid induces rapid polymerization of the polyaziridine compounds in the bath, and reduces the efficiency of the reagent. By pretreating the textile with a low concentration of mineral acid prior to impregnation with the polyaziridine, the catalytic effect of the acid can be achieved without impairing the stability of the treating solution, and without reducing the effectiveness of the reagent by initiating a polymerization reaction prior to contacting the reagent with the protein fiber.

When the process of this invention is employed to treat woolen textiles, it can be carried out on the woolen material prior to dyeing. Alternatively the process of this invention can be carried out after dyeing, as the finishing step, or at intermediate stages of processing.

The procedure employed for the evaluation of the aziridine compounds as shrinkproofing agents and feltproofing agents for keratin fibers was as follows. Samples of wool flannel of various types were treated on a laboratory padder with aqueous solutions of the selected reagent, framed to the original dimensions and dried at moderate temperature (160° to 200° F.) in a laboratory oven. After drying, the reaction was allowed to proceed under varying conditions of temperature for varying periods of time. The samples were then washed at 100°-110° F. in a mild detergent solution to remove residual unreacted material, framed to the original dimensions and dried. Control samples were handled in identical manner, except that no reagent was used in the padding solution. Untreated controls were also included in the evaluation.

The evaluation of initial fabric properties included the observation of appearance and handle and the determination of tensile strength (Ravel strip method ASTM-D-39-59). The samples were then subjected to repeated launderings (full cycle at 105° F.) in a home-type washing machine, with tumble drying or pressing between launderings. The surface appearance of the fabric samples, and the shrinkage were determined at intervals. Felting and shrinkage of the untreated controls and of the water controls were extremely severe. The treatments invariably reduced the shrinkage and felting, but some compounds proved much more efficient and effective than others in achieving control of shrinkage and felting without producing undesirable side effects.

The present invention will be more completely understood by reference to the following examples which illustrate the differences noted above between the untreated controls and fabrics treated by the novel process of this invention. Moreover, it is also apparent that the polyaziridines corresponding to the generic Formulas III and IV above are the most desirable and effective reagents. In each instance all parts and percentages are by weight unless otherwise specified.

## EXAMPLE 1

70 Reagent:



## TREATMENT

| Wool Sample No. | Conc. Pad Solution, Percent Reagent | Catalyst         | Reaction Time and Temp. | Percent Wt. Increase | Tensile St. Warp Lbs. | Remarks        |
|-----------------|-------------------------------------|------------------|-------------------------|----------------------|-----------------------|----------------|
| A               | 10                                  | None             | 24 hrs. <sup>1</sup>    | 7.4                  | 21                    |                |
| B               | 8                                   | do               | 24 hrs. <sup>1</sup>    | 6.0                  | 21                    |                |
| C               | 6                                   | do               | 24 hrs. <sup>1</sup>    | 4.8                  | 21                    |                |
| D               | 4                                   | do               | 24 hrs. <sup>1</sup>    | 4.0                  | 22                    |                |
| E               | 2                                   | do               | 5' at 300° F            | 2.1                  | 20                    |                |
| F               | 6                                   | ( <sup>1</sup> ) | 5' at 300° F            | 5.2                  | 21                    |                |
| G               | 4                                   | ( <sup>1</sup> ) | 5' at 300° F            | 2.6                  | 20                    |                |
| H               | 2                                   | ( <sup>1</sup> ) | 5' at 300° F            | 2.1                  | 22                    |                |
| Control (1)     | 0                                   | None             |                         |                      | 21                    | Untreated.     |
| Control (2)     | 0                                   | ( <sup>1</sup> ) |                         |                      | 22                    | Catalyst only. |

<sup>1</sup> Fabric pretreated with aqueous solution of 1% sulfuric acid and dried.<sup>2</sup> Room temperature.

## EVALUATION

[Samples tumble dried after each laundering]

| Wool Sample No. | Percent Area Shrinkage |      | Remarks          |
|-----------------|------------------------|------|------------------|
|                 | 1L                     | 5L   |                  |
| A               | 0.5                    | 1.5  | No felting.      |
| B               | 1.5                    | 1.9  | Do.              |
| C               | 0.5                    | 2.3  | Do.              |
| D               | 0.0                    | 1.6  | Do.              |
| E               | 1.8                    | 2.5  | Do.              |
| F               | 1.8                    | 2.9  | Do.              |
| G               | 2.3                    | 3.6  |                  |
| H               | 3.5                    | 5.4  |                  |
| Control (1)     | 14.6                   | 29.5 | Extreme felting. |
| Control (2)     | 9.7                    | 23.0 | Do.              |

There was no discoloration and no harshening of those fabric samples which were treated with low concentration of reagent and reacted at room temperature (samples B through E). More severe conditions (samples A, F to H) resulted in a slight harshening of hand which essentially disappeared in the course of tumble drying.

## EXAMPLE 2

Reagent:



## TREATMENT

| Wool Sample No. | Conc. Pad Solution percent Reagent | Catalyst         | Reaction Time and Temp. | Percent Wt. Increase | Tensile St. Warp Lbs. | Remarks          |
|-----------------|------------------------------------|------------------|-------------------------|----------------------|-----------------------|------------------|
| A               | 8                                  | None             | 20 hrs. RT <sup>2</sup> | 4.6                  | 46                    |                  |
| B               | 6                                  | do               | 20 hrs. RT <sup>2</sup> | 3.8                  | 45                    |                  |
| C               | 4                                  | do               | 20 hrs. RT <sup>2</sup> | 3.3                  | 46                    |                  |
| D               | 2                                  | do               | 20 hrs. RT <sup>2</sup> | 1.4                  | 44                    |                  |
| E               | 4                                  | ( <sup>1</sup> ) | 5' at 300° F            | 2.3                  | 47                    | Some harshening. |
| F               | 2                                  | ( <sup>1</sup> ) | 5' at 300° F            | 1.3                  | 46                    |                  |
| Control (1)     | 0                                  | None             |                         |                      | 44                    | Untreated.       |
| Control (2)     | 0                                  | ( <sup>1</sup> ) |                         |                      | 45                    | Catalyst only.   |

<sup>1</sup> Fabric pretreated with aqueous solution of 1% sulfuric acid and dried.<sup>2</sup> Room temperature.

## EVALUATION

[Samples tumble dried after each laundering]

| Wool Sample No. | Percent Area Shrinkage |      | Remarks               |
|-----------------|------------------------|------|-----------------------|
|                 | 1L                     | 5L   |                       |
| A               | 0.0                    | 1.5  | No felting.           |
| B               | 0.0                    | 2.5  | Do.                   |
| C               | 1.5                    | 8.4  | Slight felting.       |
| D               | 2.0                    | 9.7  | Do.                   |
| E               | 5.7                    | 7.8  | Do.                   |
| F               | 8.6                    | 11.6 | Considerable felting. |
| Control (1)     | 22.0                   | 49.5 | Extreme felting.      |
| Control (2)     | 17.5                   | 40.0 | Do.                   |

## EXAMPLE 3

Reagent:



## TREATMENT

| Wool Sample No. | Conc. Pad Solution, Percent Reagent | Catalyst         | Reaction Time and Temp. | Percent Wt. Increase | Tensile St. Warp, Lbs. | Remarks                   |
|-----------------|-------------------------------------|------------------|-------------------------|----------------------|------------------------|---------------------------|
| A               | 8                                   | None             | 3' at 300° F            | 5.3                  | 43                     | Slight harshening.        |
| B               | 6                                   | do               | 24 hrs. RT <sup>2</sup> | 4.3                  | 41                     | Soft hand.                |
| C               | 4                                   | do               | 24 hrs. RT <sup>2</sup> | 2.1                  | 40                     | Do.                       |
| D               | 2                                   | do               | 24 hrs. RT <sup>2</sup> | 1.5                  | 42                     |                           |
| E               | 4                                   | ( <sup>1</sup> ) | 5' at 300° F            | 2.6                  | 42                     |                           |
| F               | 2                                   | ( <sup>1</sup> ) | 24 hrs. RT <sup>2</sup> | 1.0                  | 41                     |                           |
| Control (1)     | 0                                   | None             |                         |                      | 41                     |                           |
| Control (2)     | 0                                   | ( <sup>1</sup> ) |                         |                      | 40                     | Untreated. Catalyst only. |

<sup>1</sup> Fabric pretreated with 1% aqueous solution of sulfuric acid and dried.<sup>2</sup> Room temperature.

## EVALUATION

[Samples tumble dried after each laundering]

| Wool Sample No. | Percent Area Shrinkage |      | Remarks                           |
|-----------------|------------------------|------|-----------------------------------|
|                 | 1L                     | 5L   |                                   |
| A               | 0.0                    | 0.0  |                                   |
| B               | 0.0                    | 0.5  | Perfect surface after laundering. |
| C               | 1.0                    | 2.0  | Do.                               |
| D               | 5.0                    | 31.0 |                                   |
| E               | 2.0                    |      |                                   |
| F               | 3.5                    |      |                                   |
| Control (1)     | 22.0                   | 49.5 | Extreme felting.                  |
| Control (2)     | 17.5                   | 40.0 | Do.                               |

## EXAMPLE 4

Reagent:



## TREATMENT

| Wool Sample No. | Conc. Pad Solution, Percent Reagent | Catalyst         | Reaction Time and Temp. | Percent Wt. Increase | Tensile St. Warp, Lbs. | Remarks                                                                   |
|-----------------|-------------------------------------|------------------|-------------------------|----------------------|------------------------|---------------------------------------------------------------------------|
| A               | 10                                  | None             | 24 hrs. RT <sup>2</sup> | 5.5                  | 43                     |                                                                           |
| B               | 8                                   | do               | 10' at 250° F           | 4.75                 | 42                     |                                                                           |
| C               | 6                                   | do               | 24 hrs. RT              | 3.5                  | 41                     |                                                                           |
| D               | 6                                   | ( <sup>1</sup> ) | 5' at 300° F            | 4.25                 | 42                     | All samples somewhat harsher than untreated become soft after first wash. |
| E               | 4                                   | ( <sup>1</sup> ) | 24 hrs. RT              | 3.0                  | 42                     |                                                                           |
| Control (1)     | 0                                   | None             |                         |                      | 41                     | Untreated.                                                                |
| Control (2)     | 0                                   | ( <sup>1</sup> ) |                         |                      | 42                     | Catalyst only.                                                            |

<sup>1</sup> Fabric pretreated with 1% aqueous solution of sulfuric acid and dried.<sup>2</sup> Room temperature.

## EVALUATION

[Samples tumble dried after each laundering]

| Wool Sample No. | Percent Area Shrinkage |      | Remarks          |
|-----------------|------------------------|------|------------------|
|                 | 1L                     | 5L   |                  |
| A               | 0.0                    | 0.5  | No felting.      |
| B               | 0.5                    | 2.5  | Do.              |
| C               | 1.0                    | 6.9  | Do.              |
| D               | 5.0                    | 17.7 |                  |
| E               | 9.5                    | 21.0 |                  |
| Control (1)     | 22.0                   | 49.5 | Extreme felting. |
| Control (2)     | 17.5                   | 40.0 | Do.              |

## EXAMPLE 5

Reagent:



## TREATMENT

| Wool Sample No. | Conc. Pad Solution, Percent Reagent | Catalyst  | Reaction Time and Temp. | Percent Wt. Increase | Tensile St. Warp, Lbs. | Remarks     |
|-----------------|-------------------------------------|-----------|-------------------------|----------------------|------------------------|-------------|
| A.....          | 15                                  | None..... | 20 hrs RT <sup>1</sup>  | 8.7                  | 40                     |             |
| B.....          | 7.5                                 | do.....   | 20 hrs RT <sup>1</sup>  | 5.6                  | 39                     |             |
| C.....          | 3.75                                | do.....   | 20 hrs RT <sup>1</sup>  | 2.7                  | 41                     |             |
| D.....          | 1.9                                 | do.....   | 5' at 280° F            | 1.7                  | 41                     |             |
| Control.....    | 0                                   | do.....   |                         |                      | 40                     | Water only. |

<sup>1</sup> Room temperature.

## EVALUATION

[Samples tumble dried after each laundering]

| Wool Sample No. | Percent Area Shrinkage |      | Remarks |
|-----------------|------------------------|------|---------|
|                 | 1L                     | 5L   |         |
| A.....          | 0.0                    | 0.5  |         |
| B.....          | 0.0                    | 1.5  |         |
| C.....          | 0.5                    | 3.0  |         |
| D.....          | 3.5                    | 22.6 |         |
| Control.....    | 17.0                   | 52.4 |         |

## EXAMPLE 6

With the bis-aziridine



the results obtained are essentially identical to those shown above in Example 5.

## EXAMPLE 7

Reagent:



## TREATMENT

| Wool Sample No. | Conc. Pad Solution, Percent Reagent | Catalyst         | Reaction Time and Temp. | Percent Wt. Increase | Tensile St. Warp, Lbs. | Remarks     |
|-----------------|-------------------------------------|------------------|-------------------------|----------------------|------------------------|-------------|
| A.....          | 10                                  | None.....        | 8 hrs. RT <sup>1</sup>  | 6.7                  | 42                     |             |
| B.....          | 8                                   | do.....          | 8 hrs. RT               | 5.0                  | 43                     |             |
| C.....          | 6                                   | do.....          | 18 hrs. RT              | 4.3                  | 41                     |             |
| D.....          | 4                                   | do.....          | 18 hrs. RT              | 3.5                  | 44                     |             |
| E.....          | 2                                   | do.....          | 18 hrs. RT              | 2.5                  | 41                     |             |
| F.....          | 6                                   | ( <sup>1</sup> ) | 5' at 300° F            | 4.1                  | 42                     |             |
| G.....          | 4                                   | ( <sup>1</sup> ) | 5' at 300° F            | 2.1                  | 41                     |             |
| H.....          | 2                                   | ( <sup>1</sup> ) | 5' at 300° F            | 1.3                  | 40                     |             |
| Control.....    | 0                                   | None.....        |                         |                      | 41                     | Water only. |

<sup>1</sup> Fabric pretreated with 1% aqueous solution of sulfuric acid and dried.<sup>2</sup> Room temperature.

## EVALUATION

[Samples tumble dried after each laundering]

| Wool Sample No. | Percent Area Shrinkage |      | Remarks                         |
|-----------------|------------------------|------|---------------------------------|
|                 | 1L                     | 5L   |                                 |
| A.....          | 0.5                    | 2.9  | No noticeable felting.          |
| B.....          | 1.5                    | 3.5  | Do.                             |
| C.....          | 1.5                    | 3.6  | Do.                             |
| D.....          | 2.5                    | 5.4  | Do.                             |
| E.....          | 3.5                    | 9.3  | Slight felting.                 |
| F.....          | 0.5                    | 2.2  | No felting, but some harshness. |
| G.....          | 1.5                    | 2.1  | Do.                             |
| H.....          | 4.5                    | 11.6 | Some felting and harshness.     |
| Control.....    | 18.0                   | 56.5 | Extreme felting.                |

When the experiment described in Example 7 was repeated using other types of woolen fabrics, and fabrics containing wool blended with synthetic fibers (for example a wool/nylon or a wool/polyester fabric), similar excellent results were obtained. When the treated samples were pressed after each laundering (rather than tumble dried), shrinkage and felting were completely eliminated even after 5 launderings.

## EXAMPLE 8

The following series of experiments was carried out in order to compare the effectiveness of the polyaziridines corresponding to generic Formulas III and IV (and demonstrated by the treatments of Examples 1 to 7) with the effectiveness of polyaziridine compounds corresponding to generic Formulas I and II. In these experiments, samples of woolen flannel were treated with a 5%-6% solution of the aziridine compound by padding (no catalyst was used), framed to the original dimensions, dried at 160°-180° F., reacted at room temperature for 24 hours, washed, and dried on frames. The shrinkage was then determined by the procedure outlined above *after 5 launderings*. The samples were pressed after each laundering.

Table I

|        | Compound Applied                                                                    | Generic Formula      |
|--------|-------------------------------------------------------------------------------------|----------------------|
| a..... | Reagent of example 2                                                                | IV<br>(equation 6))  |
| b..... | Reagent of example 7                                                                | III<br>(equation 3)) |
| c..... |  | II<br>(equation 1))  |
| d..... |  | II<br>(equation 4))  |
| e..... |  | II<br>(equation 5))  |
| f..... |  | I                    |
| g..... |  | I                    |
| h..... | Commercial resin <sup>1</sup>                                                       |                      |
| .....  | None (Untreated Control)                                                            |                      |

<sup>1</sup> A nitrogenous-formaldehyde resin sold as a shrinkproofing agent for wool under the trade mark Lanaset by the American Cyanamid Co. It was applied according to the manufacturer's recommendations.

Table II

|        | Percent Weight Increase | Percent Area Shrinkage | Remarks                                                               |
|--------|-------------------------|------------------------|-----------------------------------------------------------------------|
| 20     |                         |                        |                                                                       |
| a..... | 3.4                     | 0.5                    |                                                                       |
| b..... | 2.2                     | 1.5                    |                                                                       |
| c..... | 3.1                     | 2.5                    |                                                                       |
| 25     |                         |                        |                                                                       |
| d..... | 4.6                     | 2.8                    | Reagent prepared from glutaraldehyde and ethylene imine.              |
| e..... | 3.0                     | 4.5                    | Reagent prepared from divinyl sulfone and ethylene imine.             |
| 30     |                         |                        | Reagent prepared from ethylene glycol bisacrylate and ethylene imine. |
| f..... | 1.4                     | 14.8                   | Amido aziridine.                                                      |
| g..... | 2.0                     | 26.5                   |                                                                       |
| h..... | 2.0                     | 35.0                   | (1).                                                                  |
| l..... |                         | 49.5                   |                                                                       |

<sup>1</sup> A nitrogenous-formaldehyde resin sold as a shrinkproofing agent for wool under the trade mark Lanaset by the American Cyanamid Co. It was applied according to the manufacturer's recommendations.

35 It is apparent from the experiments described in this example that amino aziridines are generally more effective shrinkproofing agents for wool than amido aziridines. Even the less effective polyaziridines, however, decreased the shrinkage more significantly than a commercial resin applied by the recommended procedure.

40

15

## EXAMPLE 9

Several monoaziridine compounds were applied to woolen fabric in order to study their effect on the shrinkage and felting. The following compounds were used:



Although the above monoaziridine compounds reacted with the fiber in excellent yields, as indicated by the weight increase, they did *not* significantly improve the dimensional stability of the fabric. The results of these experiments indicate that polyfunctionality and cross-linking are required for effective shrinkage control of woolen fabrics with aziridine compounds.

While the illustrative embodiments of the invention have been described hereinbefore with particularity, it will be understood that various other modifications will be apparent to and can readily be made by those skilled in the art without departing from the scope and spirit of the invention. Accordingly, it is not intended that the scope of the claims appended hereto be limited to the examples and description set forth herein but rather that the claims be construed as encompassing all the features of patentable novelty which reside in the present invention including all features which would be treated as patentable equivalents thereof by those skilled in the art to which the invention pertains.

I claim:

1. A process of improving the dimensional stability of proteinaceous materials comprising reacting said materials with polyfunctional aminoaziridine compounds corresponding to the structure:



in which R<sub>1</sub>, R<sub>2</sub>, and R<sub>3</sub> are selected from the group consisting of hydrogen and lower alkyl, R<sub>4</sub> is selected from the group consisting of hydrogen, lower alkyl and OH, and A is selected from the group consisting of alkylene, hydroxy-substituted alkylene, aralkylene, oxyalkylene, sulfone-containing alkylene, and the residue of a carboxylic acid ester, the valence of which is equal to n and n has a value of 2 to 3.

2. The process of claim 1 wherein the proteinaceous material is a keratin fiber.

3. The process of claim 1 wherein the polyaziridine compound corresponds to the structure:



16

in which R<sub>1</sub>, R<sub>2</sub> and R<sub>3</sub> are selected from the group consisting of hydrogen and lower alkyl, m has a value of 2 to 4, and x has a value of 1 to 50.

4. The process of claim 1 wherein the polyaziridine compound corresponds to the structure:



5. The process of claim 1 wherein the polyaziridine compound corresponds to the structure:



6. The process of claim 1 wherein the polyaziridine compound corresponds to the structure:



7. The process of claim 1 wherein the polyaziridine compound corresponds to the structure:



8. The process of claim 1 wherein the polyaziridine compound corresponds to the structure:



9. The process of claim 1 wherein the proteinaceous material consists at least in part of woolen fiber in fiber, thread, yarn or fabric form.

10. The process of claim 9 wherein the reaction between the wool and the aminoaziridine compound is carried out by impregnating the wool with aqueous solution of the reagent, drying and thereafter allowing the reaction to proceed until essentially complete.

11. The process of claim 9 wherein the reaction between the wool and the aminoaziridine compound is carried out by impregnating the wool with an aqueous solution of the reagent, drying and thereafter allowing the reaction to proceed at temperatures ranging from ambient to 350° F. until essentially complete.

12. The process of claim 9 wherein the wool is used in the form of fabric.

13. The product of claim 1.

14. The fabric prepared in accordance with claim 10.

15. The process of improving the dimensional stability of proteinaceous materials comprising reacting said materials with polyaminoaziridine compounds corresponding to the structure:



wherein R<sub>1</sub>, R<sub>2</sub> and R<sub>3</sub> are selected from the group consisting of hydrogen and lower alkyl, and R represents an alkylene group.

16. The process of improving the dimensional stability of proteinaceous materials comprising reacting said mate-

trials with polyaminoaziridine compounds corresponding to the structure:



wherein  $R_1$ ,  $R_2$  and  $R_3$  are selected from the group consisting of hydrogen and lower alkyl, and  $R$  represents an alkylene group.

17. The process of improving the dimensional stability of proteinaceous materials comprising reacting said materials with polyaminoaziridine compounds corresponding to the structure:



wherein  $R_1$ ,  $R_2$ ,  $R_3$  are selected from the group consisting of hydrogen and lower alkyl,  $R_4$  is selected from the group consisting of hydrogen and methyl,  $b$  has a value of 0 to 1, and  $R^e$  is an organic radical containing conjugated unsaturation.

18. The process of claim 1 wherein the polyamino-aziridine compound corresponds to the structure:



19. The process of claim 1 wherein the polyaziridine compound corresponds to the structure:



20. The process of improving the dimensional stability of proteinaceous materials comprising reacting said materials with polyaminoaziridine compounds corresponding to the structure:



wherein  $R_1$ ,  $R_2$  and  $R_3$  are selected from the group consisting of hydrogen and lower alkyl, and  $R$  is selected from the group consisting of aralkylene and alkylene groups.

**References Cited in the file of this patent**

UNITED STATES PATENTS

- 2,831,018 Trieschmann ----- Apr. 15, 1958  
 2,889,289 Reeves et al. ----- June 2, 1959  
 2,911,325 Drake et al. ----- Nov. 3, 1959